



CHARLES M. ROWLEY, OF CHICAGO, ILLINOIS.

*Letters Patent No. 87,793, dated March 16, 1869.*

**IMPROVED PREPARATION FOR POLISHING METALLIC SURFACES.**

The Schedule referred to in these Letters Patent and making part of the same.

*To all whom it may concern:*

Be it known that I, CHARLES M. ROWLEY, of Chicago, in the county of Cook, and State of Illinois, have invented a new and improved Preparation for Polishing Metallic Surfaces; and I do hereby declare that the following is a full and exact description thereof.

The nature of my invention consists in the preparation of a polishing-fluid, by the combination of hydrochloric acid, sulphuric acid, and pumice-stone, with or without the addition of borax and fullers' earth.

For ordinary use, I prepare a mixture of hydrochloric acid, sulphuric acid, and pumice-stone, by diluting one part, by weight, of oil of vitriol with twenty parts of water, and adding one part of the dilute acid obtained to one part of dilute hydrochloric acid, made by adding six to ten parts of water to one part of common hydrochloric acid, and then adding the pumice-stone, in fine powder, and in the proportion of one part to eight parts of the mixed dilute acids.

These proportions are not essential, but may be varied greatly, without detriment, provided only great dilution be maintained. I add to the above, one part

of fullers' earth and one-sixteenth of a part of borax, in cases where there is grease to be removed, or where the best effect is desired, and where the expense is not an objection.

The advantage and usefulness of this invention are in the fact that the most rapid and effective polishing and cleaning-action is obtained upon the greatest variety of metallic surfaces, owing to the combination of the two acids, aided by the mechanical action of the pumice-stone and the grease-removing action of the borax and the fullers' earth.

I am aware that these acids, and also pumice-stone, have separately been used for similar purposes; but

What I claim, is—

The combination of the acids above described with the polishing-powder above described, with or without the borax and fullers' earth, also above described, the same being used for the purposes specified.

CHARLES M. ROWLEY.

Witnesses:

W. H. BULLOCK,  
G. A. MARINER.